

K. R. R. SEIFERT,  
COMBINED SINTERING AND STRETCHING PROCESS.  
APPLICATION FILED APR. 21, 1913.

1,103,382.

Patented July 14, 1914.



Witnesses:  
R. Kuehne,  
John Herr

Karl R. R. Seifert  
Inventor  
By his Attorney  
Ivan E. Koenigsker

# UNITED STATES PATENT OFFICE.

KARL R. R. SEIFERT, OF CHARLOTTENBURG, GERMANY.

## COMBINED SINTERING AND STRETCHING PROCESS.

1,103,382.

Specification of Letters Patent.

Patented July 14, 1914.

Application filed April 21, 1913. Serial No. 762,484.

To all whom it may concern:

Be it known that I, KARL R. R. SEIFERT, a citizen of the German Empire, and a resident of Charlottenburg, Berlin, Germany, have invented certain new and useful Improvements in Combined Sintering and Stretching Processes, of which the following is a specification.

This invention relates to a method of and apparatus for the combined sintering and stretching of wolfram, titanium, tantalum, uranium and other metals and their alloys having a high fusion point.

The object of the invention is to devise a process in which the said metals or their alloys may be sintered and stretched by means of an electric current.

Another object of the invention is to provide an apparatus for the carrying out of the process.

Before being sintered and stretched the crystals or finely divided particles of the metal or alloy have been compressed or otherwise formed into rods or ingots of suitable size preparatory to their further treatment, which heretofore have involved the use of a great deal of machinery such as electric furnaces, swaging, hammering and rolling machines before being acted upon by the well known wire drawing machinery which produces the fine wires for filaments, resistances or other uses. The known manner of treating the metals or their alloys necessarily involves a great deal of time and expense and causes considerable waste.

The object of my invention, as stated above, is to provide a single apparatus in which the combined process of sintering and stretching may be carried out in a simple and practical manner and with little expenditure of time and labor and at a comparatively low cost.

The invention is embodied in an apparatus for carrying out the process and which is described in detail in the following specification while reference is had to the accompanying drawing, which is to be understood as illustrating the preferred form of the apparatus but not as showing the only form in which my invention may be embodied.

In the drawing, Figure 1 is a vertical sectional view of an apparatus for carrying out my process of combined sintering and stretching. Fig. 2 is a detail view illus-

trating a step in the process. Fig. 3 is a detail view of a water cooled die used in the apparatus and Fig. 4 illustrates the process diagrammatically.

Referring to the drawing the reference numeral 5 represents a suitable base for the machine and in which is secured a die support 6. The die support 6 is provided with a socket 7 into which is laid a die holder 8 through the opening 9. The die holder 8 contains the die frame 11 in which is supported a die 12 of suitable material, such as a hard stone for instance, or as shown in Fig. 3, I may prefer a hollow hard steel die 50 provided with means as 51 for water cooling. 13 is the opening in the die. The aforesaid parts are preferably cylindrical and the die frame 11 is removably held in the die holder to facilitate the exchange of dies as will be pointed out later.

Into the die support 6 there are screwed pipes 14 and 15 generally of metal, and these pipes are lined with sleeves 16 of insulating material. End pieces or holding means 17 of insulating material are secured at the outer ends of the pipes 14 and 15 and provided with apertures forming bearings or guiding means 18 for the electrodes 19 and 20 to which current is supplied by means of cables 21 secured to clamping means 22 of conducting material and clamped to the said electrodes as shown. The electrodes are movable lengthwise within the sleeves 16 through the bearings 18. If desired, other suitable guiding means may be provided.

The electrodes 19 and 20 consist of hollow pipes of suitable material such as copper for instance and are provided with means for securing the metal ingot between them.

In the drawing such means are illustrated and may comprise for the electrode 19 a pair of jaws 23 pivoted to a conducting holder 24 secured in the end of the electrode. 25 is a sleeve which may be moved to cause the jaws to close as will be understood.

A holder 26 is provided in the electrode 20. The holder has a conical head 27 or other means for causing the jaws 28 to close by expanding them on one side of their pivot 29.

The electrodes are hollow and water cooled. Water is admitted through the pipes 30 into the interior of the electrodes and passes out through the pipes 31. Suitable

reducing gases are admitted within the sleeves 16 through the pipes 32 and pass out through the pipes 33, 34 is a claw member which fits over the head 35 of the electrode 20, but is insulated therefrom by a member 36, 37 is a swivel eye to which is attached a cable or other pulling means 38.

Stated briefly, the operation consists in securing the ingot 40 of the metal between 10 the electrodes, heating the ingot to cause it to sinter and drawing the ingot through the die to stretch it. The ingots have a diameter of about 8 mm., and are stretched to a diameter of about 1 mm., these dimensions, 15 however, not being absolute or controlling.

Describing the process in detail, the ingot 40 is shaped at one end so as to pass through a die having a die opening of less diameter than the ingot which is gripped by the jaws 20 28 as seen in Fig. 2. The other end of the ingot is caught between the jaws 23 and the sleeve 25 is moved out over the jaws to secure the ingot. Then the current is turned on and passes through the electrodes and the 25 ingot 40, thus heating the latter. At the same time water is admitted to the electrodes to cool them and reducing gases are admitted through the pipes 32 to prevent oxidation of the ingot during the process. A 30 current of about 1000 to 1500 amperes, more or less depending upon the fusibility of the metal and the dimensions thereof, is sent through the ingot and causes it to sinter by the action of the heat and simultaneously 35 therewith the stretching process commences by pulling on the cable 38 by suitable means to draw the hot ingot through the die and whereby the ingot is reduced in diameter. The harder the pull on the electrode 20, the 40 harder the ingot is clamped between the jaws 28 because of the cone-shaped head 27. As the electrode moves out through the bearing 18 the ingot is stretched through the die and the pulling power will be transmitted to the 45 electrode 19 which will move to the right also until the sleeve 25 abuts the die holder. Continued pull frees the jaws 23 from the sleeve and the metal will be stretched and drawn through the die and the current will 50 be automatically broken. Thereafter the apparatus is taken apart, a die having a smaller die opening is inserted, the ingot is again secured to the electrodes, a current of sufficient amperage is sent through the ingot 55 to heat and further sinter it and the ingot is again stretched through the die. Then again the apparatus is taken apart, a still smaller die is inserted, the ingot, which gradually has assumed the shape of a rod, is 60 again heated by a proportionately reduced current and stretched, and so the operation is repeated until the rod of metal has been reduced to a diameter of about 1 mm. more or less.

65 The process of reducing the ingot by sin-

tering and stretching through the repeated operation as described is shown diagrammatically in Fig. 4 in which an ingot 60 is shown as having been reduced to a rod 61 by heating and passing it through a die 62; and the rod 61 is shown as being still further reduced to a rod 63 by being stretched through a die 64 having a smaller opening than the die 62, and the rod 63 is shown finally reduced to a very thin rod 65 by being stretched through a die 66 of less die opening than the die 64.

Fig. 4 does not illustrate the entire operation or process, but only three stages thereof. The operation of sintering and stretching the rod through the various sized dies is repeated as often as is necessary until a rod of the required thinness has been obtained. Further, it will be understood and is a feature of my invention, that with each reduction in diameter of the metal, the current is correspondingly reduced. Also, that I may at each stage of the process either heat the metal to sinter it and simultaneously therewith stretch the metal, or I may at certain 90 shown finally reduced to a very thin rod 65 by being stretched through a die 6 of less die opening than the die 64.

From the foregoing it will be seen that my invention provides a process whereby an 95 ingot or rod of metal is reduced in diameter from one given dimension to another given dimension by a combined process of sintering and stretching, by means of an electric current and by repetitions of the process, in 100 which each stage is similar to another stage except that the amperage of the current is proportionately reduced as the metal is reduced in diameter by passing it through the dies of varying die openings.

It will be seen that the apparatus described is of very simple construction and easily operated. The pipes 14 and 15 which form a sintering chamber are quickly detached from the die support 6 by unscrewing the pipes and the dies may readily be changed as they are removably held in the die frame as shown.

The form of the apparatus as illustrated is susceptible of changes within the principle of invention and I do not wish to limit myself otherwise than as demanded by the scope of the appended claims.

I claim:

1. The method of sintering and stretching 120 wolfram or other metals and their alloys which consists in sintering the metal by means of an electric current, stretching the metal by passing it through a suitable die and subjecting the metal during the sintering and stretching process to the influence of reducing gases.

2. The method of sintering and stretching 125 wolfram or other metals and their alloys which consists in sintering the metal by 130

means of an electric current and simultaneously therewith stretching the metal by passing it through a suitable water cooled die.

3. The method of sintering and stretching 5 wolfram or other metals and their alloys which consists in sintering the metal by means of an electric current and simultaneously therewith stretching the metal by passing it through a suitable water cooled die, 10 and subjecting the metal during the sintering and stretching process to the influence of reducing gases.

4. The method of sintering and stretching 15 wolfram or other metals and their alloys which consists in subjecting the metal to the action of an electric current to sinter it and simultaneously therewith treating the metal mechanically to stretch it.

5. The method of sintering and stretching 20 wolfram or other metals and their alloys which consists in passing an electric current through the metal to sinter it and stretching the metal by passing it through a suitable die while the current is on.

25 6. The method of sintering and stretching wolfram or other metals and their alloys which consists in heating the metal to sinter it and simultaneously therewith reducing the diameter of the metal by mechanical means.

30 7. The method of sintering and stretching wolfram or other metals and their alloys which consists in securing the metal between two electrodes, sintering the metal by passing a continuous electric current through it 35 and the electrodes and operating the latter to stretch the metal simultaneously with the sintering thereof.

8. The method of sintering and stretching 40 wolfram or other metals and their alloys which consists in passing one end of the metal through a die, securing the metal between two electrodes, one on each side of said die, sintering the metal by passing an electric current through it and simultaneously 45 therewith stretching the metal by passing it through the said die.

9. The method of sintering and stretching 45 wolfram or other metals and their alloys which consists in heating the metal to sinter 50 it, stretching the metal by passing it through a mechanical reducing means while maintaining the heat and subjecting the material to the influence of reducing gases during the entire process.

55 10. An apparatus for the combined sintering and stretching of wolfram or other metals and their alloys comprising two electrodes, means for securing the metal or alloy between the same, means for passing an

electric current through said electrodes and 60 the metal or alloy, a die and means for mechanically operating said electrodes to stretch the metal or alloy through the said die.

11. An apparatus for the combined sintering and stretching of wolfram or other metals and their alloys comprising two electrodes, means for securing the metal or alloy between the electrodes, a die, means for operating the electrodes to stretch the metal 70 through the said die and means for passing continuous electric current through the metal or alloy while the same is being stretched.

12. An apparatus for the combined sintering and stretching of wolfram or other 75 metals and their alloys comprising a cylinder, a die in the same, two electrodes supported one on each side of said die, means for securing the metal or alloy between said electrodes, means for passing an electric current through said electrodes and metal or alloy, means for operating the electrodes to stretch the metal or alloy through the die, means for cooling the electrodes and means for admitting reducing gases to said cylinder. 80

13. An apparatus for the combined sintering and stretching of wolfram or other metals and their alloys comprising a support, a die removably held in said support, cylinders removably secured to the latter to both 90 sides of said die, end pieces secured to the outer ends of said cylinders, electrodes movably supported in said end pieces, means for passing an electric current through said electrodes, means for cooling the latter and means for admitting reducing gases to the 95 said cylinders.

14. An apparatus for the combined sintering and stretching of wolfram or other metals and their alloys comprising a center support, a die in the same, pipes removably secured to said support to form cylinders to both sides of the die, an electrode movably supported in each cylinder, means at the 105 inner ends of the electrodes for securing the metal or alloy between them, means at the outer ends of the electrodes for passing an electric current through them and mechanism connected to one of said electrodes for 110 operating the electrode lengthwise of the cylinder in which the electrode is supported.

Signed at New York, N. Y. this 17th day of April 1913.

KARL R. R. SEIFERT.

Witnesses:

K. G. LEARD,  
HERMAN LUDWIG GYNE.